

Patented May 23, 1939

2,159,643

# UNITED STATES PATENT OFFICE

2,159,643

## METHOD FOR PRODUCING CELLULOSE ESTERS

Richard Weingand and Ernst Acker, Bomlitz,  
near Walsrode, Germany, assignors to Sylvania  
Industrial Corporation, Fredericksburg, Va., a  
corporation of Virginia

No Drawing. Application November 10, 1937, Se-  
rial No. 173,862. In Sweden May 4, 1935

8 Claims. (Cl. 260—222)

The invention relates in general to cellulose derivatives and, in particular, to a process for the preparation of a cellulosic raw material adapted to be used in the preparation of cellulose derivatives and to correlated improvements designed to enhance the properties and usefulness of the products so produced.

In making cellulose esters it is customary to use cellulose in the form of thick paper boards with a weight of about 500 g. per square meter and with a specific gravity of about 0.6. When employing such cellulose boards for the esterification, there are great difficulties due to the fact that the cellulose swells only to a small degree. For instance, when esterifying cellulose boards by means of the known nitrating mixture consisting of sulphuric acid, nitric acid and water, a superficial nitration of cellulose board takes place shortly after their introduction into the esterifying liquid. The nitrocellulose layer which is formed in this way at the surface inhibits the penetration of the mixed acid into the inner parts of the cellulose board and the removal of the water liberated during the nitration. In view thereof, it is hardly possible, even with a longer duration of nitration to obtain a final product which is uniformly nitrated throughout the mass.

In order to avoid these drawbacks it has already been proposed to form the cellulose, by means of a paper machine, into very thin paper sheets having a weight of about 20 to 30 g. per square meter. Furthermore, these paper sheets are creped in order to prevent the several nitrated sheets from adhering together and to enable the acid to penetrate between the different sheets. The formation of cellulose into such thin creped sheets is expensive and even with such sheets a relatively large quantity of mixed acid is required for the nitration in comparison with the quantity of acid necessary for nitrating an equivalent quantity of cotton linters. Furthermore, the creped paper occupies in the nitration receptacle a relatively large volume due to its creped condition and, therefore, the capacity of an existent nitration plant becomes considerably reduced in comparison with the treatment of cotton linters.

Therefore, it is a general object of the invention to overcome the above mentioned disadvantages of the prior art and to produce cellulose derivatives having improved properties from a cellulosic raw material prepared in a simple and economical manner.

It is a further object of the invention to provide a cellulosic raw material having improved properties which make it especially adapted for the preparation of cellulose derivatives.

It is another object of the invention to provide a process for making cellulose derivatives from a cellulosic raw material of such physical and

chemical character that the properties of the cellulose derivative so produced are improved and the cost diminished.

It is a specific object of the invention to provide a process of making nitrocellulose from a cellulosic raw material of the above mentioned characteristics.

According to the invention, cellulose derivatives of improved properties are prepared using as raw material a cellulose of high alpha cellulose content prepared by treating wood fibres first with a relatively dilute alkali at an elevated temperature and pressure to disintegrate the cellulose fibres and separate the non-cellulose substances therefrom, and thereafter refining the disintegrated fibres by treatment with a relatively concentrated alkali at atmospheric temperature and pressure to remove as by dissolving the non-cellulose constituents without substantially mercerizing the cellulose, and purifying the product in a known manner. The purified cellulose fibres are felted into a sheet on a suitable paper machine without exercise of substantial pressure either during sheeting or during drying to produce a substantially undegraded cellulose of above 93% alpha cellulose in the form of a thin sheet having a loose porous structure, a specific gravity of form not above 0.4 and an absorptivity for water of not substantially above 200 seconds.

The purified alpha cellulose in the form of a thin porous sheet of the above mentioned characteristics may be converted to cellulose derivatives, such as cellulose ethers and esters, in a known manner. In particular, a nitrocellulose suitable for gun cotton may be made by nitration of the paper sheet with a suitable acid, the product being stabilized and converted into explosive materials in a suitable manner.

The invention accordingly comprises a process having the several steps and the relation of one or more of such steps with respect to each of the others thereof and a purified cellulose sheet possessing the features, properties and the relation of constituents which are exemplified in the following detailed disclosure, and the scope of the invention will be indicated in the claims.

As raw material for use in preparing cellulose derivatives according to the invention, there may be employed any suitable cellulosic material of vegetable origin, in particular, wood pulp, such as spruce, pine and the like. The wood fibres are first disintegrated and separated by treating the wood pulp with a dilute aqueous solution of a strong alkali at an elevated temperature and elevated pressure. For example, wood pulp may be treated with an aqueous solution containing from about, per liter, 7.5% to 9.0% of sodium hydroxide and 1.5% to 2.0% of sodium sulfide. Preferably, the amount of alkali per weight of dry wood pulp is from about 18% to 20%, not including the

amount of sodium sulfide as black liquor which may be added thereto. The disintegrating treatment is carried out at an elevated temperature, for example, at about 170° C. and at an elevated pressure, for example, at 8 atmospheres, the treatment taking place in a suitable pressure chamber. After several hours' treatment there is obtained a product which comprises chiefly ligno cellulose, the treatment having removed the incrustations of the wood, such for example, as lignin, hemi-celluloses, sugar, resins, fats and other non-cellulosic constituents of the pulp. During this alkali treatment the fibres are separated one from another, but they are not substantially gelatinized nor is the cellulose substantially degraded.

The disintegrated fibres are subjected to an alkali refining treatment designed to remove the non-cellulose substances from the fibres by dissolution. This second alkali treatment is characterized by employing a relatively concentrated aqueous solution containing from 9% to 20% of a strong alkali. The ratio of solid alkali to dry cellulose in this treatment is about 7 to 1. The treatment is carried out at atmospheric pressures and at a temperature such that the cellulose fibres are not substantially mercerized or gelatinized. Using an aqueous solution of 10% sodium hydroxide, a temperature of from 16° C. to 20° C. is suitable. During this alkali refining treatment, the non-cellulose substances, such as, lignin, pentosans, resin and fats are removed. The product may be washed with water and treated with suitable mineral acid to neutralize the residual alkali. After centrifuging there is obtained an undegraded cellulose pulp comprising from 93% to 95% alpha cellulose.

This purified alpha cellulose pulp may be subjected to a bleaching treatment, if desired. For example, the alkali-purified cellulose may be bleached with an aqueous solution of sodium hypochlorite containing about 20 g. of free chlorine per liter, the temperature of the bleaching solution being about 35° C. to 40° C. The bleached product is then well washed to remove the bleaching agent.

To prepare the wood pulp for esterification, it is preferable to form it into a thin paper sheet of loose porous structure. For sheeting the pulp, there may be employed a long sieve paper machine or a paper machine of the cylinder sieve type. During the sheeting the paper is carried through the machine without subjecting it to any substantial pressure so as to avoid compacting the sheet. The wet sheet is then dried over a suitable drier which does not subject the sheet to substantial pressure. By avoiding substantial pressure during both sheeting and drying there is produced a paper sheet which is characterized by having a loose porous structure, a specific gravity of not above 0.3 to 0.4 and an absorptivity for esterification acids of from 40 to 200 seconds. It is preferable to sheet the material in such a manner that the dried sheet has a thickness of about 1.5 mm., although the invention is not to be limited to sheets of such thickness.

The absorption time is a measurement of the time required for water to travel by capillary action between two spaced points on a paper strip, one end of which is immersed in water. To determine the absorption time, a cellulose strip having a width of 20 mm., a length of 100 mm. and a thickness of 1.5 mm. is provided with three marks positioned at distances of 10 mm.,

15 mm., and 65 mm., respectively, from the lower edge. This strip is dipped vertically into water up to the lower mark and the time required for the water to rise from the middle to the upper mark is measured.

The sheet of interfelted cellulose fibres of the present invention is especially adapted for conversion to various cellulose derivatives, such as cellulose ethers, for example, methyl cellulose, ethyl cellulose, and cellulose esters, for example, cellulose nitrate, cellulose acetate, and the like, in a suitable manner.

For example, the porous, highly absorptive purified cellulose sheets may be cut into small pieces having the area of about the palm of the hand. After a short preliminary drying, these pieces are treated at a temperature of 15° C. to 20° C. for 30 minutes with a nitrating mixture composed of 23 per cent nitric acid, 67% sulphuric acid and 10 per cent water, the quantity of mixed acids being about forty or fifty times the weight of the dry cellulose. After a suitable period of treatment the main quantity of the nitrating acid is eliminated by means of a hydro-extractor and the acid still adhering is removed by washing the nitrocellulose. The nitrocellulose may be stabilized by treatment with hot water. The major quantity of water is eliminated by means of a centrifugal separator to such a degree that the nitrocellulose contains about 35 per cent water. By varying the conditions of nitration and the ratio and concentration of the acids, there may be produced nitrocellulose adapted for use in plastics, collodions, lacquers, explosives, etc.

For example, to produce smokeless powder, a gun cotton nitrocellulose obtained by means of this invention and having about 13.3 per cent nitrogen, will be mixed with a quantity of collodion fibres necessary for the gelatination and made of a nitrocellulose containing about 12.3 per cent nitrogen. These collodion fibres are produced in a manner analogous to the manufacture of gun cotton nitrocellulose by nitrating the same initial material, that is to say, loose porous cellulose sheets by means of a suitable nitrating acid. Water is extracted from the mixture of gun cotton and collodion fibres by means of alcohol. Then, the mixture is introduced into a kneading machine where it is mixed with ether and transformed into a gelatinized plastic mass. The shaping of this mass is effected in the usual manner by extruding the mass through a suitable orifice. For instance, for the production of smokeless powder, there are employed orifices of rectangular cross section, whereby narrow flat bands are obtained, and these bands are transformed, after partial removing of the solvents, into the small leaves as customary.

It is known that hemi-celluloses are decomposed to a large extent by esterifying acids. Therefore, the removal of the hemi-cellulose as effected by the present invention prevents the contamination of the esterifying acids, so that a higher yield of the desired cellulose derivatives is obtained with a smaller quantity of acid. Moreover, when the present alkali purification treatments are prolonged, there is obtained a product having an alpha cellulose content above 93% with which the yield of nitrocellulose is greater, and the consumption of the acid less than with the sulphite cellulose of the prior art. Further, the purer alpha cellulose gives clearer solutions of the cellulose esters produced therefrom.

Since the alkali-purification treatment of the present invention is carried out without substantial mercerization, gelatinization or degradation of the alpha cellulose, the cellulose esters produced from such purified cellulose are equal to or better than those prepared directly from cotton linters. In particular, the less degraded cellulose of the invention produces a nitrocellulose of higher specific gravity and gives products, such as films, etc., of greater strength than those made from sulphite cellulose.

By avoiding pressure during sheeting and drying of the purified cellulose pulp, the absorptivity of the sheets produced by the invention is greatly increased. The loose porous structure of the present sheet avoids the formation of superficial layers of cellulose ester on the sheet so that penetration of the esterifying acids is rapid and uniform throughout the sheet. In addition, the porous structure of the present sheet decreases the quantity of acid which remains adhering to the cellulose after squeezing and extraction of the acid, in consequence of which less acid is wasted in washing.

A further advantage of the loose porous structure of the present sheet is the fact that the absorption of the acid is very rapid, so that there is no need to crepe the sheet of the present invention as is necessary with those produced with sulphite cellulose of the prior art. By using the uncreped porous sheet of the invention the capacity of an esterification apparatus is fifty per cent greater than when creped sheets are employed.

Since certain changes in carrying out the above process, and certain modifications in the article which embody the invention may be made without departing from its scope, it is intended that all matter contained in the above description shall be interpreted as illustrative and not in a limiting sense.

This application is a continuation in part of our application Serial No. 20,690 filed May 9, 1935.

We claim:

1. A process which comprises treating cellulose wood fibres with relatively dilute alkali containing from about 7½ to 9% alkali at an elevated temperature and pressure to disintegrate the wood fibres and to separate non-cellulose components therefrom, thereafter treating said disintegrated fibres with a relatively concentrated alkali containing from about 9 to 20% alkali at atmospheric temperature and pressure to remove the non-cellulose components from the fibres, forming said fibres into a sheet without subjecting said sheet to substantial pressure during sheeting and drying.

2. A process which comprises treating cellulose wood fibres with relatively dilute alkali containing from about 7½ to 9% alkali at an elevated temperature and pressure to disintegrate the wood fibres and to separate non-cellulose components therefrom, thereafter treating said disintegrated fibres with a relatively concentrated alkali containing from about 9 to 20% alkali at atmospheric temperature and pressure to remove the non-cellulose components from the fibres, forming said fibres into a sheet without subjecting said sheet to substantial pressure during sheeting and drying to form a product having an absorptivity for water of not substantially more than 200 seconds.

3. A process which comprises treating cellu-

lose wood fibres with relatively dilute alkali containing from about 7½ to 9% alkali at an elevated temperature and pressure to disintegrate the wood fibres and to separate non-cellulose components therefrom, thereafter treating said disintegrated fibres with a relatively concentrated alkali containing from about 9 to 20% alkali at atmospheric temperature and pressure to remove the non-cellulose components from the fibres, forming said fibres into a sheet without subjecting said sheet to substantial pressure during sheeting and drying and converting the said sheet into cellulose derivatives.

4. A process which comprises treating cellulose wood fibres with relatively dilute alkali containing from about 7½ to 9% alkali at an elevated temperature and pressure to disintegrate the wood fibres and to separate non-cellulose components therefrom, thereafter treating said disintegrated fibre with a relatively concentrated alkali containing from about 9 to 20% alkali at atmospheric temperature and pressure to remove the non-cellulose components from the fibres, felting said fibres into a sheet without subjecting it to substantial pressure during sheeting and drying to produce a sheet having an absorptivity of not less than 200 seconds and converting said sheet into cellulose nitrate.

5. A process for making cellulose esters comprising esterifying a sheet of inter-felted substantially undegraded cellulose fibres substantially free of non-cellulosic constituents having a thickness of about 1.5 mm., a loose porous structure, a specific gravity of from 0.3 to 0.4 and an absorptivity for water of from 40 seconds to 200 seconds and produced in accordance with claim 1.

6. A process for making cellulose nitrate comprising nitrating a sheet of inter-felted substantially undegraded cellulose fibres substantially free of non-cellulosic constituents and having a thickness of about 1.5 mm., a loose porous structure, a specific gravity of from 0.3 to 0.4 and an absorptivity for water of from 40 second to 200 seconds and produced in accordance with the process of claim 1.

7. A sheet of inter-felted substantially undegraded cellulose fibres substantially free of non-cellulosic constituents and having a thickness of about 1.5 mm., a loose porous structure, a specific gravity of from 0.3 to 0.4 and an absorptivity for water of from 40 seconds to 200 seconds produced in accordance with the process of claim 1.

8. The process for producing a sheet of inter-felted cellulosic fibres adapted for conversion into cellulose derivatives, comprising treating cellulose wood fibres with an alkali solution having a concentration of from 7.5% to 9% by weight at elevated temperature and pressure, the amount of alkali being sufficient to give a ratio of solid alkali to cellulose of 1:5, to disintegrate the wood fibres and to separate non-cellulose components therefrom, thereafter treating said disintegrated fibres with an alkali solution having a concentration of from about 9% to 20% by weight at atmospheric pressure and temperature, the ratio of solid alkali to cellulose being from 0.7 to 1, to remove the non-cellulose components from the fibre and forming said treated fibres into a sheet without subjecting the fibres to substantial pressure during sheeting and drying.

RICHARD WEINGAND.  
ERNST ACKER.